

## [54] INHIBITOR COATING FOR SOLID ROCKET PROPELLENT CHARGE

[75] Inventor: Eduard Daume, Richterswil, Switzerland

[73] Assignee: Werkzeugmaschinenfabrik Oerlikon-Bührle AG, Zurich, Switzerland

[21] Appl. No.: 587,322

[22] Filed: June 16, 1975

## [30] Foreign Application Priority Data

June 21, 1974 Switzerland 8518/74

[51] Int. Cl.<sup>2</sup> F42B 1/00

[52] U.S. Cl. 102/103; 149/2

[58] Field of Search 149/2, 19.4; 102/103

## [56] References Cited

## U.S. PATENT DOCUMENTS

|           |        |                |            |
|-----------|--------|----------------|------------|
| 3,144,830 | 8/1964 | DeFries et al. | 102/103    |
| 3,447,980 | 6/1969 | Voigt          | 149/19.4   |
| 3,529,042 | 9/1970 | Lippert        | 149/19.4 X |
| 3,554,820 | 1/1971 | Evans          | 149/19.4   |

|           |         |                    |            |
|-----------|---------|--------------------|------------|
| 3,682,727 | 8/1972  | Heinzelmann et al. | 149/19.4 X |
| 3,714,047 | 1/1973  | Marion et al.      | 102/103 X  |
| 3,716,604 | 2/1973  | Dehm               | 102/103 X  |
| 3,813,308 | 5/1974  | Skidmore           | 149/109    |
| 3,855,176 | 12/1974 | Skidmore           | 102/103 X  |

Primary Examiner—Edward A. Miller  
 Attorney, Agent, or Firm—Werner W. Kleeman

## [57] ABSTRACT

An inhibitor coating for a solid propellant charge for protecting against undesired burning-off, comprising:

- a. an insulating layer containing a binder and a filler, and
- b. a protective- and adhesion layer located between the insulating layer and the propellant charge;
- c. the binder consisting of a castable mass which has poor smoke developing properties;
- d. the filler consisting of a fine granular cooling agent possessing good packability; and
- e. the protective- and adhesion layer consisting of a completely set polyisocyanate forming a barrier against plasticizer migration.

5 Claims, No Drawings

## INHIBITOR COATING FOR SOLID ROCKET PROPELLENT CHARGE

### BACKGROUND OF THE INVENTION

The present invention relates to a new and improved inhibitor coating or the like for solid propellant charges for protecting against undesired burning-off, the inhibitor coating comprising an insulating layer containing a binder and a filler and a protective- and adhesion layer which is located between the insulating layer and the propellant charge.

Inhibitor coatings of this type are known to the art by means of which there is covered a portion of the surface of the propellant charge in order to protect such surfaces against undesired burn-off. This measure is necessary when the rocket propellant charges are freely exposed within the rocket combustion chamber, especially when the propellant charge is constructed as an internal burner or an end burner. In both cases the effective burning surface of the propellant charge is determined by the reliable insulation of the remaining surfaces of the propellant charge. An undesired burn-off or burning-off at such insulated surfaces owing to detachment or failure of the insulating layer leads to ballistic malfunctions or tearing-down of the rocket and must be prevented.

### REQUIREMENTS WHICH ARE PLACED UPON THE COATING

The following requirements are placed upon the quality of the inhibitor coating or covering:

- a. The coating must be capable of withstanding temperature fluctuations in a range between -40° C to +60° C, i.e., it is either elastic or it possesses the same coefficient of expansion as the propellant charge.
- b. The coating must be capable of withstanding the mechanical and thermal loads during the burn-off, for instance, the acceleration forces during the flight of the rocket.
- c. The coating must be capable of being removed in as gaseous state as possible during the burning-off, since larger proportions of carbon black particles or other solid particles lead to the pronounced formation of smoke, something which must be absolutely avoided in the case of wire-guided rockets.
- d. The coating must not decompose or disintegrate into larger pieces or parts, since otherwise such parts can clog the nozzles.

### COMPOSITION OF THE COATING

These prior art inhibitor coatings can contain:

- a. an organic binder formed of plasticized or nonplasticized elastomeric or elastomeric polymers,
- b. inorganic or organic fillers,
- c. fabrics formed of polymeric organic or inorganic substances, for instance formed of polyesters or glass which can be wound about the propellant charge.

### MANUFACTURE AND APPLICATION OF THE COATING

These inhibitor coatings are applied by immersing the propellant charge in an insulating bath, by coating, by pressing-on, casting or by adhesively bonding skins or hides. The momentarily employed manufacturing technique is dictated by the composition of the binder.

### THE DRAWBACKS AND DIFFICULTIES OF THE STATE-OF-THE-ART COATINGS

- a. Coatings containing elastomeric binders, e.g., ether and ester derivatives of cellulose can only be applied in a dissolved state as a lacquer by immersion, coating or spraying.
- b. There can be only applied relatively thin layers, so that there are necessary the application of a number of layers and hence there must be carried out a number of working operations or steps because between the working steps there must take place each time a drying and removal of the solvent.
- c. The migration of the plasticizer cannot be prevented, so that over prolonged periods of time the coating is softened and impaired in its effectiveness.
- d. The winding of foils about the propellant charge, and which foils have been imbued with the aforementioned lacquer, is cumbersome. When adhesively binding skins or hides the danger exists that such will not adequately adhere at localized regions, particularly at the seam.
- e. Filled or unfilled coatings with elastomeric binders such as, for instance, polyurethanes, unsaturated polyesters or polyepoxides must be processed within the so-called "pot life", i.e., at the beginning of the hardening phase. Such coatings can only be applied by casting or pressing-on. The technique of pressing-on the coating is associated with the drawback that the working speed is small.

### SUMMARY OF THE INVENTION

It is a primary object of the present invention to produce and apply an inhibitor coating possessing the following beneficial properties:

- a. there can be employed casting or pouring techniques,
- b. slight development of smoke,
- c. good mechanical properties,
- d. good adhesion to the surface of the solid propellant charge.

### DETAILED DESCRIPTION OF THE INVENTION

Now in order to implement the foregoing object, and others which will become more readily apparent as the description proceeds, the invention contemplates a new and improved inhibitor coating which is manifested by the following features:

- a. the binder consists of a castable mass which possesses poor smoke developing properties,
- b. the filler consists of a fine grain or fine granular cooling agent possessing good packability or densification, and
- c. the protective- and adhesion layer consists of a completely set or cure hardened polyisocyanate forming a barrier against plasticizer migration.

The inhibitor coating which is composed in this manner effectively solves the above-stated objectives.

### A. USEFUL FOR CASTING TECHNIQUES

The casting technique requires mixtures possessing good flow properties. This requirement is fulfilled by means of the binder which is used, and due to the limitation of the largest possible proportion of a fine grain filler possessing high packability. By virtue of the foregoing there is of course limited the formulation possibility. However, this limitation is advantageously compensated by the advantages prevailing when employing

casting techniques, to wit, high production speeds, simplicity of the method.

### B. SMALL DEVELOPMENT OF SMOKE

Systematic experiments regarding the influence of the binder composition upon the development of smoke or fumes have shown that in particular aromatic compounds constitute the primary cause for the disturbing development of smoke or the like. All further experiments or tests therefore were directed towards producing highly-filled, but still castable insulation mixtures containing a pronounced aliphatic binder.

### A. THE FILLERS

The fillers have the function of improving the insulating properties of the inhibitor coating. The proportion of filler is limited both by the workability of the mass employed for the insulating layer as well as also by the mechanical properties of the mixture.

It is known to use as the filler inorganic substances possessing low thermal conductivity, for instance, asbestos, mica, and quartz in powder form.

Furthermore, there are used cooling agents, that is to say, solid inorganic or organic compounds, which at elevated temperatures markedly endothermically decompose into gaseous products, and thus, cool their surroundings.

For instance, there are used compounds containing water of crystallization, such as aluminum sulfate, aluminum fluoride, lithium metaborate, magnesium sulfate, sodium silicate or ammonium salts containing water of crystallization or free from water of crystallization, such as ammonium oxalate, ammonium sulfate, ammonium borate or compounds which easily decompose such as urea or melamine.

Due to the large proportion of cooling agent in the insulating layer it is possible to:

- a. improve the insulating properties,
- b. reduce the quantity of coarse carbonization products, which result from organic binders,
- c. reduce the formation of smoke,
- d. avoid clogging of the nozzles.

The cooling agents are more suitable than the inert fillers. The cooling agent should be present in a granulometric form of high packability, so that with good casting or pouring properties there is possible a high volumetric proportion of filler.

When speaking in terms of the packability of a dispersed filler there is to be understood the proportion by volume of the pure filler with complete compaction by jarring or shaking. The packability  $P$  is the quotient of the shaking density  $\rho_R$  and the filler density  $\rho$ . This can be expressed by the following equation:

$$P = \frac{\rho_R}{\rho}$$

As the cooling agent there is particularly suitable aluminium hydroxide,  $\text{Al(OH)}_3$ , possessing a density equal to  $2.41 \text{ g/cm}^3$  and a shaking density equal to  $1.500$  to  $1.545 \text{ g/cm}^3$ .

With such aluminium hydroxide,  $\text{Al(OH)}_3$ , there can be realized still good castable insulating layers with a proportion of 60 to 62 percent by weight filler.

### B. THE BINDER

The binder is preferably composed of an isocyanate-containing polyether pre-adduct, a diamine hardener and an aliphatic plasticizer.

On the one hand, in order to be able to lower the viscosity of this pre-adduct to a degree required for the casting process, and, on the other hand, to reduce the aromatic proportion to such an extent that with slight formation of smoke there is still insured for satisfactory adhesion, there are undertaken the following measures:

a. Complete reaction of the pre-adduct with an aromatic diamine and the addition of an aliphatic plasticizer.

b. Complete reaction of the pre-adduct with a stoichiometric mixture of an aromatic diamine and a higher molecular triol.

### C. THE PROTECTIVE- AND ADHESION LAYER

Between the solid propellant charge and the insulating layer there is located a protective layer which initially must be applied to the propellant charge. For this protective layer there is preferably employed a completely moisture-hardened, low-molecular weight triisocyanate.

This protective layer has the following functions:

a. To improve the adhesion of the insulating layer at the propellant charge owing to its high concentration of urea groups formed from free isocyanate and atmospheric moisture.

b. To form a barrier against the migration of the plasticizer owing to its high degree of cross-linking due to the tri-functionality and the small molar or molecular mass.

This barrier functions in both directions in the event that both the insulating layer as well as also the propellant charge contains plasticizer. The second property is important since the plasticizer migration in the one or the other direction constitutes the cause of the impairment — which becomes increasingly more pronounced as a function of time — of the adhesion of the coating at the propellant charge until complete detachment of the coating from the propellant charge.

For this protective layer there is especially suitable the following triisocyanate:

triphenylmethane - 4,4',4''-triisocyanate.

The lacquer-technological properties can be improved by the addition of additives, for instance 30 to 100 percent by weight of butyl acetate to the prepared 20%-solution in methyl chloride of the aforementioned triisocyanate.

This improvement can be readily proven or ascertained by virtue of the good anchoring of the protective layer at the propellant charge and a good wetting, leading to a homogeneous film formation.

In order to transform the protective layer applied by spraying, coating or immersion into a defined condition, i.e., into a completely set or cured condition, within a useful period of time, the propellant charges provided with a protective layer are subjected for approximately 15 hours to a temperature of  $60^\circ \text{C}$  and a relative humidity of 70 to 90%. Consequently, the wetting process — which at room temperature and depending upon the humidity of the air lasts for 1 to 3 weeks — can be shortened.

**D. DESCRIPTION OF TWO EXEMPLARY EMBODIMENTS OF THE INVENTION**

The invention will be now described in greater detail in conjunction with two exemplary embodiments discussed hereinafter.

**EXAMPLE 1**

The propellant charge is initially coated with a protective- and adhesion layer. This layer consists of a solution of:

20 parts by weight triphenylmethane- 4,4',4''-triisocyanate

80 parts by weight methylene chloride

30 parts by weight butyl acetate.

The solution must then be applied in a thin condition. After an evaporation time of 1 hour the protective layer is cured or hardened for 15 hours at 60° C in a moist atmosphere, preferably in an air circulating oven or furnace with closed air valves and with a vessel filled with water located in the oven compartment or chamber.

Thereafter there is applied an insulating layer. This consists of a mixture containing:

223.6 grams of a polyether-pre-adduct possessing an isocyanate content of 4.3% as hardener.

156 grams acetyltri-n-butyl-citrate.

This mixture is degassed and dewatered in a kneader for half an hour at 70° C and a pressure of about 1 mm Hg pressure (Torr).

Thereafter there is added to the mixture the following:

780 grams of aluminium hydroxide as the filler.

Granulation size <150  $\mu$ .

Packability 62%.

This mixture is then admixed or stirred for half an hour under the same conditions.

Thereafter there is added to the mixture the following:

40.4 grams molten 4,4'-methylene-bis-[2-chloroaniline] as the hardener.

The new mixture is again processed for 5 minutes in the kneader and subsequently applied to the propellant charge. For this purpose the propellant charge is placed into a casting mold, so that there is formed a 2 mm thick hollow space between the casting mold and propellant charge into which there is poured the aforementioned mixture. The propellant charge consists of a double base-propellant grain or powder and possesses a diameter of 100 mm. The inner surface of the coating mold is provided with a "TEFLON" coating. After curing or hardening for 10 hours at 60° C the propellant charge provided with the coating can be removed from the casting mold.

After undergoing temperature-alternating tests of 6 cycles at -50° C to +60° C such processed propellant charge displayed no changes in the adhesion of the coating.

Stand burn-off in test chambers with nozzles of large flow constriction took place without disturbances both

5 with tested as well as untested propellant charges at extreme temperatures of -40° C and +60° C.

Smoke measurements produced results in the order of less than 8 dB.

**EXAMPLE 2**

The protective layer is the same as that described with respect to the first exemplary embodiment of Example 1.

Thereafter there is applied the insulating layer. This consists of a mixture containing the following:

364.2 grams of a polyether-pre-adduct possessing an isocyanate content of 6.5%.

155.8 grams of a hardener solution consisting of 22.4 grams 4,4'-methylene-bis-[2-chloroaniline], 133.4 grams castor oil possessing an hydroxide content of 5%.

20 Initially the pre-adduct is degasified and dewatered in a kneader at a temperature of 70° C and a pressure of 1 mm Hg pressure (Torr), and thereafter there is added the hardener solution. After stirring or mixing for 5 minutes the mixture is filled into the mold under the same conditions as discussed above in conjunction with the first embodiment of Example 1.

25 Propellant charges provided with such coating gave the same results during all tests.

The inhibitor coatings can be composed of the following components, which more or less satisfactorily fulfill the stated objectives:

1. Filler-Cooling Agent

Aluminum hydroxide possessing a packability of 64%.

2. Binder

PU (A) Polyurethane - partially aliphatic - pre-adduct containing 4.3% content of isocyanate which is stoichiometrically crosslinked with 4,4'-methylene-bis-[2-chloroaniline].

PU (B) Polyurethane - partially aliphatic - pre-adduct containing 6.5% content of isocyanate which is stoichiometrically crosslinked with 30 Mol % NH<sub>2</sub> from 4,4'-methylene-bis-[2-chloroaniline] 70 Mol % OH from castor oil with 5% OH.

PU (C) Polyurethane - purely aliphatic - produced in a one-shot process from polyoxypropylene glycol and trimethylolpropane cross-linked with 4,4'-methylene-bis(cyclohexylisocyanate) catalyzed with

0.5% stannous dibutyl-dilaurate

0.5% iron acetyl-acetonate

Composition of the mixture in Mol % of the reactive groups of the participating partners

Diol 70

Triol 30

NCO 100

PE Soft foam unsaturated polyester, hardened by the addition of methyl ethyl-ketone peroxide and cobalt naphthanate.

WM Acetyltri-n-butyl citrate.

DPA Diphenylamine (an aromatic substance which is readily soluble in polyurethane and added for comparative purposes)

DA 4,4'-methylene-bis-[2-chloroaniline].

Table I

## Influence Of The Proportion Of Cooling Agent Upon The Development Of Smoke

| Ex. | Cooling Agent | PE | PU(A) | PU(B) | Binder |    | Aromatic Proportion | Smoke <sup>(1)</sup> |
|-----|---------------|----|-------|-------|--------|----|---------------------|----------------------|
|     |               |    |       |       | PU(C)  | WM |                     |                      |
| 4   | 60            |    | 40    |       |        |    | 7.0                 |                      |
| 3   | 45            |    | 55    |       |        |    | 10.5                |                      |

Table II

## Influence Of The Binder Composition Upon Smoke Development

| Ex. | Cooling Agent | PE | PU(A) | PU(B) | Aromatic Proportion |     | Smoke <sup>(1)</sup> |
|-----|---------------|----|-------|-------|---------------------|-----|----------------------|
|     |               |    |       |       | Binder              | WM  |                      |
| 1   | 60            | 40 |       |       |                     | 11  | 15                   |
| 2   | 45            |    | 53.5  |       | 1.5                 | 11  | 13.5                 |
| 3   | 45            |    | 55.0  |       |                     | 11  | 10.5                 |
| 4   | 60            |    | 40.0  |       |                     | 11  | 7.0                  |
| 5   | 60            |    | 28.0  |       | 12.0                | 7.8 | 6.0                  |
| 6   | 60            |    |       | 40    |                     | 4.3 | 6.0                  |
| 7   | 60            |    |       | 40    |                     | 0   | 4.3                  |

<sup>(1)</sup>The smoke measurement is given in dB, with average or mean weakening of the light during the burning-off.

Finally it is to be mentioned that all of the concentrations given herein, unless otherwise stated, are in percent by weight.

Obviously, many modifications and variations of the present invention are possible in light of the above teachings. It is, therefore, to be understood that within the scope of the appended claims the invention may be practiced otherwise than as specifically described.

What is claimed is:

1. The combination of an inhibitor coating and a solid double base propellant charge comprising:
  - a. a polyurethane protective- and adhesion layer consisting essentially of a lowmolecular weight triisocyanate applied to the propellant charge;
  - b. a castable insulating layer for protecting said propellant charge against undesired burning-off applied to said protective- and adhesion layer and comprising: (i) a binder of polyurethane, (ii) a fine granular cooling agent as filler;
  - c. said polyurethane of the insulating layer being different from the polyurethane of said protective- and adhesion layer and possessing poor smoke developing properties;
  - d. said filler containing aluminium hydroxide and possessing good packability;
  - e. said protective- and adhesion layer being completely moisture hardened by atmospheric mois-

ture before the application of the insulating layer and forming a barrier against plasticizer migration.

2. The combination as defined in claim 1, wherein the cooling agent has a grain size less than 150 microns, and the grain size is adjusted such that there is attained a packability of at least 55 percent by volume, the packability being designated by the symbol P which is the quotient of the solid density  $\rho$  in grams/cm<sup>3</sup> and the density  $\rho_R$  in grams/cm<sup>3</sup> wherein

$$P = \frac{\rho_R}{\rho}$$

3. The combination as defined in claim 1, wherein the binder of the insulating layer is cross-linked with diamine and additionally with castor oil in that the diamine is partially replaced by castor oil.

4. The combination as defined in claim 1, wherein the binder contains a plasticizer of acetyltri-n-butyl citrate.

5. The combination as defined in claim 2, wherein the grain size of the fine granular cooling agent is less than 150 microns.

\* \* \* \* \*

50

55

60

65